



US007833591B2

(12) **United States Patent**  
**Ghyzel et al.**

(10) **Patent No.:** **US 7,833,591 B2**  
(45) **Date of Patent:** **Nov. 16, 2010**

(54) **IMAGE RECORDING ELEMENT  
COMPRISING ENCAPSULATED MORDANT  
PARTICLES**

(75) Inventors: **Peter J. Ghyzel**, Rochester, NY (US);  
**Joseph F. Bringley**, Rochester, NY (US); **David J. Giacherio**, Rochester, NY (US); **Lawrence P. DeMejo**, Rochester, NY (US); **Terry C. Schultz**, Hilton, NY (US)

(73) Assignee: **Eastman Kodak Company**, Rochester, NY (US)

(\*) Notice: Subject to any disclaimer, the term of this patent is extended or adjusted under 35 U.S.C. 154(b) by 835 days.

(21) Appl. No.: **11/617,777**

(22) Filed: **Dec. 29, 2006**

(65) **Prior Publication Data**

US 2008/0160228 A1 Jul. 3, 2008

(51) **Int. Cl.**  
**B41M 5/40** (2006.01)

(52) **U.S. Cl.** ..... **428/32.34**; 428/32.26; 428/32.29;  
428/32.36; 428/32.37; 347/95; 347/105

(58) **Field of Classification Search** ..... 428/32.26,  
428/32.29, 32.34, 32.36, 32.37; 347/95,  
347/105

See application file for complete search history.

(56) **References Cited**

U.S. PATENT DOCUMENTS

3,870,663 A \* 3/1975 Clemens et al. ..... 521/147  
3,958,995 A 5/1976 Campbell et al.  
4,592,960 A \* 6/1986 Inoue et al. ..... 428/461  
5,221,713 A 6/1993 Kempner et al.  
6,045,917 A 4/2000 Missell et al.  
6,057,384 A 5/2000 Nguyen et al.

6,419,355 B1 7/2002 Bermel et al.  
6,447,111 B1 9/2002 Gallo et al.  
6,492,006 B1 12/2002 Kapusniak et al.  
6,521,342 B1 2/2003 Hutter et al.  
6,573,313 B2 6/2003 Li et al.  
6,619,797 B2 9/2003 Lawrence et al.  
6,645,582 B2 11/2003 Sadasivan et al.  
6,669,815 B1 12/2003 Sugiyama et al.  
6,753,051 B1 \* 6/2004 Landry-Coltrain et al. ..... 428/  
32.36  
6,767,638 B2 7/2004 Samaranayake  
6,818,685 B1 11/2004 Chapman  
6,969,445 B1 11/2005 Hibino et al.  
2004/0145088 A1 \* 7/2004 Patel et al. ..... 264/463  
2005/0031806 A1 2/2005 Kim et al.  
2008/0161493 A1 7/2008 Ghyzel et al.

FOREIGN PATENT DOCUMENTS

|    |             |         |
|----|-------------|---------|
| EP | 1 035 179   | 9/2000  |
| EP | 1184195     | 3/2002  |
| EP | 1288008     | 3/2003  |
| EP | 1288012     | 4/2003  |
| JP | 2006-089696 | 4/2006  |
| WO | 2005/009747 | 2/2005  |
| WO | 2005/118653 | 12/2005 |

\* cited by examiner

*Primary Examiner*—Betelhem Shewareged

(74) *Attorney, Agent, or Firm*—Chris P. Konkol; Andrew J. Anderson

(57) **ABSTRACT**

The present invention discloses an ink printing method using an image-recording element, which provides an image having excellent image quality and superior dry time, comprising insoluble cationic core-shell polymeric particles each comprising a core comprising cationic core polymer having at least 10 mole percent of a cationic mordant monomeric unit and a shell comprising hydrophilic shell polymer that is substantially less cationic than the cationic core polymer, wherein the shell is at least 10% by weight of the core.

**20 Claims, No Drawings**

## 1

**IMAGE RECORDING ELEMENT  
COMPRISING ENCAPSULATED MORDANT  
PARTICLES**

**CROSS REFERENCE TO RELATED  
APPLICATIONS**

Reference is made to commonly assigned, co-pending U.S. patent application Ser. No. 11/617,775 by Ghyzel et al., filed of even date herewith entitled "Encapsulated Mordant Particle Dispersion and Method of Preparing."

**FIELD OF THE INVENTION**

This invention relates to an ink printing method. More particularly, this invention relates to an ink printing method utilizing an ink recording element containing water dispersible core-shell polymer particles stabilized with an outer shell.

**BACKGROUND OF THE INVENTION**

In a typical inkjet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent. The solvent, or carrier liquid, typically is made up of water, an organic material such as a monohydric alcohol, a polyhydric alcohol or mixtures thereof.

The inks used in various inkjet printers can be classified as either dye-based or pigment-based. A dye is a colorant that is molecularly dispersed or solvated by a carrier medium. A commonly used carrier medium is water or a mixture of water and organic co-solvents.

An inkjet recording element typically comprises a support having on at least one surface thereof an ink-receiving or image-forming layer, and includes those intended for reflection viewing, which have an opaque support, and those intended for viewing by transmitted light, which have a transparent support.

It is well known that in order to achieve and maintain photographic-quality images on such an image-recording element, an inkjet recording element must be readily wetted so there is no puddling, i.e., coalescence of adjacent ink dots, which leads to non-uniform density, exhibit no image bleeding, exhibit the ability to absorb high concentrations of ink and dry quickly to avoid elements blocking together when stacked against subsequent prints or other surfaces, exhibit no discontinuities or defects due to interactions between the support and/or layer(s), such as cracking, repellencies, comb lines and the like, not allow unabsorbed dyes to aggregate at the free surface causing dye crystallization, which results in bloom or bronzing effects in the imaged areas, and exhibit excellent image quality, and provide image fastness or stability to avoid fade from contact with water, ozone, radiation by daylight, tungsten light, or fluorescent light, or other environmental conditions that can otherwise cause image fade or deterioration.

Of particular relevance to the present invention, an inkjet recording element that simultaneously provides an almost instantaneous ink dry time and good image stability is desirable. However, given the wide range of ink compositions and ink volumes that a recording element needs to accommodate, these requirements of inkjet recording media are difficult to achieve simultaneously.

## 2

Inkjet recording elements are known that employ porous or non-porous single layer or multilayer coatings that act as suitable image receiving or recording layers on one or both sides of a porous or non-porous support. Recording elements that use non-porous coatings typically have good image stability but exhibit poor ink dry time. Recording elements that use porous coatings typically contain colloidal particulates and have poorer image stability but exhibit superior dry times.

There are generally two types of ink-receiving layers. The first type of ink-receiving layer comprises a non-porous coating of a polymer with a high capacity for swelling and absorbing ink by molecular diffusion. Cationic or anionic substances may be added to the coating to serve as a dye fixing agent or mordant for a cationic or anionic dye. This coating is optically transparent and very smooth, leading to a high glossy "photo-grade" receiver. The swellable binder forms a barrier to air-borne pollutants that otherwise may degrade the image dye over time. However, with this type of ink-receiving layer, the ink is usually absorbed slowly into the ink-receiving layer and the print is not instantaneously dry to the touch. Inkjet media having a non-porous layer are typically formed of one or more polymeric layers that swell and absorb applied ink. Due to limitations of the swelling mechanism, this type of media is relatively slow to absorb the ink, but once dry, printed images are often stable when subjected to light and ozone.

The second type of ink-receiving layer comprises a porous coating of inorganic, polymeric, or organic-inorganic composite particles, a polymeric binder, and optional additives such as dye-fixing agents or mordants. These particles can vary in chemical composition, size, shape, and intra-particle porosity. In this case, the printing liquid is absorbed into the open pores of the ink-receiving layer to obtain a print that is instantaneously dry to the touch. However, with this type of ink-receiving layer, image dyes adsorbed to the porous particles are relatively exposed to air and may fade unacceptably in a short time. In other words, the ink is absorbed very quickly into the porous layer by capillary action, but the open nature of the porous layer can contribute to instability of printed images, particularly when the images are exposed to environmental gases such as ozone.

In summary, the porous inkjet recording media have excellent drying properties, but generally suffer from dye fading, whereas, the swellable type of inkjet recording media may give less dye fading, but generally dry more slowly.

There remains a need for inkjet recording media having excellent drying properties and, at the same time, showing minimal dye fading. In addition, these inkjet recording media should preferably have properties such as good image density, as well as good image quality, preferably photographic image quality. It is towards fulfilling this need that the present invention is directed.

Mordant polymer particles containing cationic groups, for use in the image-receiving layer of inkjet recording elements, in order to mordant dye-based inks, are generally well known in the art. U.S. Pat. Nos. 6,045,917 and 6,645,582, for example, disclose water-insoluble cationic polymeric particles having at least about 20 mole percent of a cationic mordant moiety. Preferred mordants comprising a polymer having a vinylbenzyl trimethyl quaternary ammonium salt moiety are disclosed. U.S. Pat. No. 6,645,582 states that such particles can be core/shell particles wherein the core is organic or inorganic and the shell in either case is a cationic polymer.

Certain types of core-shell particles have been used in inkjet recording elements. However, the prior art does not

disclose mordants in the form of core-shell particles that adequately address and solve the problem of dye fade.

U.S. Pat. No. 6,619,797 discloses an image-receiving layer comprising a cationic core/shell particle containing at least one ethylenically unsaturated monomer containing a trialkylammonium salt. However, the shell, but not the core, contains the trialkylammonium group.

U.S. Pat. No. 6,492,006 discloses an inkjet recording element comprising a support having thereon an image receiving layer comprising at least about 70% by weight of porous polymeric particles, the particles having a core/shell structure comprising a porous polymeric core covered with a shell of a water-soluble polymer. The recording element exhibited less cracking, but no improvement in dye density was disclosed. The porous polymeric particles do not have a monomer with cationic functionality, thus do not function as mordant.

US 2005/0031806 discloses a composition for forming an ink-accepting layer comprising a structured cationic core/shell latex, wherein a non-porous core does not have a cationic functional group and does not expand, and the shell contains a cationic functional group capable of expansion by an acid. The recording element exhibited improved absorption and water-fastness, but no improvement in dye fade was disclosed.

U.S. Pat. No. 6,818,685 discloses a coating composition comprising a non-ionic latex polymer (polyvinyl acetate), wherein the polyvinyl acetate has a core and a shell, and the shell comprises poly(vinyl alcohol). The particle core has no positive ionic character. A composition of high solids and low viscosity was disclosed and the recording element exhibited reduced dusting, but no improvement in dye fade as disclosed.

U.S. Pat. No. 6,969,445 and U.S. Pat. No. 6,669,815 describe graft copolymers of poly(vinyl alcohol) with cationic polymers.

#### SUMMARY OF THE INVENTION

It is an object of this invention to improve inkjet media image stability by providing a mordant with a protective barrier that, after an image is printed on the media, will shield mordanted dyes from environmental factors that will reduce stability. The present invention is especially advantageous for porous media and dye-based printing, since improving ozone stability of dye-based prints with porous media is especially problematic. Thus, an object of this invention to provide a porous inkjet recording element that when printed simultaneously provides good image stability and excellent dry time, as well as superior optical densities.

These and other objectives of the present invention are accomplished by an inkjet recording element comprising a support having thereon at least one porous image-receiving layer comprising:

(a) inorganic or organic particles (other than the below mentioned insoluble cationic core-shell polymer particles) in the amount of greater than 50 percent by weight, preferably between 60 and 95 percent by weight of the image-receiving layer; and

(b) insoluble cationic core-shell polymeric particles each comprising a core and shell, a core comprising insoluble swellable cationic core polymer having at least 10 mole percent of a cationic mordant monomeric unit and a shell comprising hydrophilic shell polymer that is substantially less cationic than the insoluble swellable cationic core polymer, wherein the shell is at least 10% by weight of the core, and the weight ratio of the insoluble cationic core-shell polymeric

particles to inorganic particles in the image-receiving layer is 1:2 to 1:30, preferably 1:3 to 1:20, more preferably 1:4 to 1:10.

Preferably, the hydrophilic shell polymer is at least 50 percent less cationic than the insoluble swellable cationic core, in terms of number of cationic groups per weight average molecular weight of the polymer, and more preferably the hydrophilic outer shell polymer is essentially non-ionic and non-cationic.

10 The porous inkjet recording element of the invention provides superior optical densities, good image quality and stability, and has an excellent dry time.

Another aspect of the present invention relates to an ink printing method comprising the steps of: A) providing an inkjet printer that is responsive to digital data signals; B) loading the inkjet printer with the inkjet recording element comprising the insoluble cationic, polymeric core-shell particles as described above; C) loading the inkjet printer with an inkjet ink; and D) printing on the inkjet recording element 20 using the inkjet ink in response to the digital data signals.

In describing the invention herein, the following definitions generally apply:

The term "porous layer" is used herein to define a layer that is characterized by absorbing applied ink by means of capillary action to a significant extent. An inkjet recording element having one or more porous layers, preferably substantially all layers, over the support can be referred to as a "porous inkjet recording element," even though at least the support is not considered porous.

30 Particle sizes referred to herein, unless otherwise indicated, are median particle sizes as determined by light scattering measurements of diluted particles dispersed in water, as measured using photon correlation spectroscopy (PCS) or MIE scattering techniques employing a NANOTRAC (Microtac Inc) ultrafine particle analyzer or a Horiba LA-920 instrument, respectively.

As used herein, the terms "over," "above," "upper," "under," "below," "lower," and the like, with respect to layers in inkjet media, refer to the order of the layers over the 40 support, but do not necessarily indicate that the layers are immediately adjacent or that there are no underlying layers.

In regard to the present method, the term "image-receiving layer" is intended to define a layer that can be used as a dye-trapping layer, or dye-and-pigment-trapping layer, in 45 which the printed image substantially resides throughout the layer. Preferably, an image-receiving layer comprises a mordant for dye-based inks. The image may optionally reside in more than one image-receiving layer.

In regard to the present method, the term "sump layer" or 50 "ink-carrier-liquid receptive layer" is used herein to mean a layer, under the upper image-receiving layer, that absorbs a substantial amount of ink-carrier liquid. In use, a substantial amount, preferably most, of the carrier fluid for the ink is received in the one or more ink-carrier-liquid receptive layers. An ink-carrier-liquid receptive layer is not above an image-containing layer and is not itself an image-containing layer (a pigment-trapping layer or dye-trapping layer). Preferably, in the case of a single ink-carrier-liquid receptive layer, the layer is an ink-receptive layer that is immediately 55 adjacent the support, not including subbing layers or the like that are not significantly absorbent.

The term "ink-receptive layer" or "ink-retaining layer" 60 includes any and all layers above the support that are receptive to an applied ink composition, that absorb or trap any part of the one or more ink compositions used to form the image in the inkjet recording element, including the ink-carrier fluid and/or the colorant, even if the former removed by drying. An

ink-receptive layer, therefore, can include an image-receiving layer, in which the image is formed by a dye and/or pigment, a porous ink-carrier-liquid receptive layer, or any additional layers, for example between a porous underlying layer and a topmost layer of the inkjet recording element.

Typically, all layers above the support are ink-receptive. The support on which ink-receptive layers are coated may also absorb ink-carrier fluid, in which it is referred to as an ink-absorptive or absorbent layer rather than an ink-receptive layer.

The term "non-ionic" is defined herewith as a polymer having essentially no cationic or anionic groups in salt form, less than 1 mole percent in terms of monomer content.

The term "swellable" is defined herewith as the polymer particle absorbs water but does not dissolve. A common method of converting an otherwise soluble polymer to a swellable polymer is to lightly crosslink it. In such polymer particles, the content of monomers with crosslinking ability is less than 110 mole percent, preferably less than 5 mole percent, and the particle is dispersible in water.

#### DETAILED DESCRIPTION OF THE INVENTION

The present mordant can be considered as having a core-shell structure having a protective shell or barrier, in which the core comprises an insoluble cationic latex having a high cationic charge concentration, relative to the shell, which core is encapsulated or surrounded by a protective shell that has a relatively low, or absence of, cationic charge, relative to the core.

Without wishing to be bound by theory, it is believed that the shell polymer, in effect, acts as a barrier against transmission of oxygen or ozone and, hence, exhibits a relatively low transmission rate for oxygen or ozone gas.

The insoluble cationic core-shell polymeric particles, each comprising a core and shell, a core comprising insoluble swellable cationic core polymer having at least 10 mole percent, preferably at least 20 mole percent, more preferably 35 to 99 mole percent, of a cationic mordant monomeric unit, most preferably greater than 50 mole percent. Preferably, a crosslinking monomer is present in the core in an amount of 0.5 to 15 mole percent, preferably 1 to 10 mole percent.

The core in the water-insoluble cationic core-shell polymeric particles comprises at least about 10 mole percent of a cationic mordant moiety. The core polymer can be the product of addition or condensation polymerization, or a combination of both. They can be branched, hyper-branched, grafted, random, blocked, or can have other polymer microstructures well known to those in the art, in addition to being crosslinked. They are insoluble or made insoluble by slightly or partially crosslinking the polymer. In a preferred embodiment, the core in the water-insoluble cationic core-shell polymeric particles comprises at least about 50 mole percent of a cationic mordant moiety. In the core polymer used to make the particles, precursor groups may be present that are later converted to cationic mordant moieties.

The core in the water-insoluble cationic core-shell polymeric particles useful in the invention can also comprise nonionic or anionic monomeric units in addition to cationic monomeric units. In a preferred embodiment, combinations of nonionic and cationic monomeric units are employed. In general, the amount of cationic monomeric units employed in the combination is at least about 20 mole percent.

The nonionic, anionic, or cationic monomeric units employed in the core of the water-insoluble cationic core-shell polymeric particles can include neutral, anionic or cationic derivatives of addition polymerizable monomers such

as styrenes, alpha-alkylstyrenes, acrylate esters derived from alcohols or phenols, methacrylate esters, vinylimidazoles, vinylpyridines, vinylpyrrolidinones, acrylamides, methacrylamides, vinyl esters derived from straight chain and branched acids (e.g., vinyl acetate), vinyl ethers (e.g., vinyl methyl ether), vinyl nitriles, vinyl ketones, halogen-containing monomers such as vinyl chloride, and olefins, such as butadiene.

The nonionic, anionic, or cationic monomeric units 10 employed can also include neutral, anionic or cationic derivatives of condensation polymerizable monomers such as those used to prepare polyesters, polyethers, polycarbonates, polyureas and polyurethanes.

The core of the water-insoluble cationic core-shell polymeric particles employed in this invention can be prepared using conventional polymerization techniques including, but not limited to bulk, solution, emulsion, or suspension polymerization. In a preferred embodiment of the invention, the core of the water-insoluble cationic particles has a mean 15 particle size of from about 10 to about 500 nm.

In a preferred embodiment of the invention, the core in the water-insoluble cationic core-shell polymeric particles contains a polymer having a quaternary ammonium salt moiety. In yet another preferred embodiment, the core in the water-insoluble cationic core-shell polymeric particles contains a polymer having a (vinylbenzyl)trimethyl ammonium salt moiety. In yet still another preferred embodiment, the core contains a polymer having a (vinylbenzyl)dialkyl benzyl quaternary ammonium salt moiety and/or the core comprises a mixture of a latex containing a polymer having a (vinylbenzyl)trialkyl quaternary ammonium salt moiety and a polymer having a (vinylbenzyl)dialkylbenzyl quaternary ammonium salt moiety. Preferred alkyl groups contain 1 to 6 carbon atoms, more preferably methyl or ethyl.

In a preferred embodiment the core polymer in the water-insoluble cationic core-shell polymeric particles can be represented by the following structure:



wherein:

A represents units of an addition polymerizable monomer containing at least two ethylenically unsaturated groups;

B represents units of a copolymerizable,  $\alpha,\beta$ -ethylenically unsaturated monomer;

N is the nitrogen in a quaternary amine;

R<sub>1</sub>, R<sub>2</sub>, R<sub>3</sub>, R<sub>4</sub>, and R<sub>5</sub> each independently represents a carbocyclic or alkyl group, wherein the core polymer forms an attachment to the shell polymer via the oxygens in the linking group;

M<sup>-</sup> is an anion;

x is from about 0.25 to about 15 mole percent;

y is from about 0 to about 90 mole percent;

z is from about 10 to about 99 mole percent;

w is from 10 to 80 weight percent;

u is preferably on average 1 to 3 per shell polymer; and

v is preferably greater than 75 mole percent for poly(vinyl alcohol).

Suitable monomers from which the repeating units of A are formed include divinylbenzene, allyl acrylate, allyl methacrylate, N-allylmethacrylamide, ethylene glycol dimethacrylate, etc.

B in the above formula is a unit of a copolymerizable  $\alpha,\beta$ -ethylenically unsaturated monomer, such as ethylene, propylene, 1-butene, isobutene, 2-methylpentene, etc. A preferred class of ethylenically unsaturated monomers that may be used includes the lower 1-alkenes having from 1 to about 6 carbon atoms; styrene, and tetramethylbutadiene and methyl methacrylate.

R<sub>1</sub>, R<sub>2</sub>, R<sub>3</sub>, R<sub>4</sub>, and R<sub>5</sub> in the above formula each independently represents a carbocyclic group such as aryl, aralkyl, and cycloalkyl such as benzyl, phenyl, p-methyl-benzyl, cyclopentyl, etc.; or an alkyl group preferably containing from 1 to about 20 carbon atoms such as methyl, ethyl, propyl, isobutyl, pentyl, hexyl, heptyl, decyl, etc. In a preferred embodiment, R<sub>1</sub>, R<sub>2</sub>, R<sub>3</sub>, R<sub>4</sub> and R<sub>5</sub> are methyl.

M<sup>-</sup> in the above formula is an anion, i.e., a negative ion forming an ionic radical or atom such as a halide, e.g., bromide or chloride, sulfate, alkyl sulfate, alkane or arene sulfonate, acetate, phosphate, etc.

Further examples of core polymers in the water-insoluble cationic core-shell polymeric particles are analogous to the mordant polymers found in U.S. Pat. No. 3,958,995, the disclosure of which is hereby incorporated by reference, except chemically bonded to shell polymers as disclosed herein. Specific examples of these core polymers, except for the one or more ammonium groups replaced by linking groups, for example, include:

Polymer A. Copolymer of (vinylbenzyl)trimethylammonium chloride and divinylbenzene (87:13 molar ratio)

Polymer B. Terpolymer of styrene, (vinylbenzyl)dimethylbenzylamine and divinylbenzene (49.5:49.5:1.0 molar ratio)

Polymer C. Copolymer of styrene, (vinylbenzyl)dimethyllocetyltrimonium chloride), isobutoxymethyl acrylamide and divinylbenzene (40:20:34:6 molar ratio)

As indicated above, the shell of the core-shell particle comprises a hydrophilic shell polymer that is substantially less cationic than the insoluble swellable cationic core polymer. Preferably, the hydrophilic outer shell polymer is at least 50 percent less cationic than the insoluble swellable cationic core, in terms of number of cationic groups per weight average molecular weight of the polymer. More preferably, the cationic groups are essentially absent from the hydrophilic outer shell polymer. The shell is at least 10% by weight of the core, preferably 50 to 400 percent by weight.

The shell polymer preferably comprises polymer having hydroxy, ether, amino acid, nitrile, and/or ketone groups, which are relatively polar and, hence, exhibit low compatibility for oxygen transmission. Examples include poly(vinyl alcohol), gelatin, polyacrylonitrile, and the like. In the preferred embodiment, the shell polymer is poly(vinyl alcohol) or a copolymer or derivative thereof.

Preferably, the shell polymer is selected to have a p(O<sub>2</sub>) (oxygen permeability) of less than 25 cm<sup>3</sup>·μm/m<sup>2</sup>·day·KPa, preferably less than 3, more preferably less than 1.0, most preferably ranging from 0.01 to 0.30 cm<sup>3</sup>·μm/m<sup>2</sup>·day·KPa.

Such values are available in standard reference books, for example, *Brandup and Immergut Polymer Handbook* 3d Edition. Since oxygen is a relatively non-polar molecule, non-polymer polymers such as olefins and acrylates or methacrylate in which the alkyl groups are not substituted with polar groups, for example, such polymers as polypropylene, polyethylene or poly(methyl methacrylate) homopolymer provide a relatively high rate of oxygen transmission and, therefore, do not provide an effective barrier.

It has been calculated that a protective layer made from a polymer such as poly(vinyl alcohol), or a similar derivative or copolymers thereof, and having a thickness of 10 to 100 nm, or more, is sufficiently thick to provide very high ozone stability.

In one particular embodiment, a reactive hydrophilic shell polymer containing one or more reactive linking groups is preformed. Preferably, the shell polymer has on average a relatively small number of reaction functionalities, preferably less than three per shell polymer, preferable one to two on average. In one embodiment, the shell polymer is terminated with a reactive linking group, for example an amine-terminated polymer. In another embodiment, which is easier to make, the shell polymer can have one or more reactive linking groups along its length.

One method to prepare a poly(vinyl alcohol) molecule with a reactive linking group is to derivatize a commercially available poly(vinyl alcohol) with a molecule containing both aldehyde and tertiary amine functionalities such as p-dimethylaminobenzaldehyde. The aldehyde will react with the polyvinyl alcohol and create an acetal ring group that attaches the compound to the poly(vinyl alcohol). The tertiary amine group is available to bond the poly(vinyl alcohol) to the core polymer.

In one embodiment, the linking-group-containing shell polymer can be added to a core polymer or intermediate thereof, in a reactive environment, to produce the core-shell mordant or intermediate thereof. The reactive linking group is designed to react with complementary reactive sites in the core polymer or intermediate thereof.

In another embodiment, (RPP—Reacted in the Presence of Poly(vinyl alcohol)), the core polymeric latex is prepared in the presence of the shell polymer, for example poly(vinyl alcohol) or a copolymer or derivative thereof, and chain transfer is relied upon to bond the shell polymer to the core polymer latex by abstraction of a radical from the shell polymer during polymerization. This approach, however, may allow for less synthetic control than use of a linking group on the shell polymer.

Other processes for making the core-shell particles used in the present invention will be known to the skilled artisan in addition to the examples and embodiments disclosed in detail herein.

In one preferred embodiment of the present invention, the core-shell particle is made by a process comprising the following steps:

(A) forming a polymer latex core intermediate from a reaction mixture of monomers, including a monomer comprising a precursor group that can be converted to a quaternary ammonium group;

(B) forming a linking-group-containing shell polymer by derivatizing a hydroxy-group-containing polymer [poly(vinyl alcohol)] with a linking agent that is a compound comprising both an aldehyde moiety and a tertiary amine moiety, wherein one or more acetal moieties are formed in the linking-group-containing shell polymer, each acetal formed by the reaction of the aldehyde moiety in the linking agent with two hydroxy groups in the shell polymer, wherein the tertiary amine moiety then becomes a linking group pendant from the linking-group-containing shell polymer, wherein the linking group is capable of reacting with said precursor group in the polymer latex core intermediate;

(C) reacting the linking-group-containing polymer with the polymer latex core intermediate prior to quaternization of the precursor group (for example with a trialkylamine such as trimethylamine) to create a core-shell particle intermediate, and

(D) obtaining quaternization of the core-shell particle intermediate with a tertiary amine compound to obtain a insoluble core-shell cationic polymeric particle.

Following Step (D), residual tertiary amine (for example, trimethylamine) can be removed by vacuum distillation. Following Step (D) and removal of tertiary amine, the insoluble core-shell cationic polymeric particle is preferably purified by diafiltration to remove excess sodium chloride. In the preferred embodiment, in Step (C), poly(vinyl alcohol) is derivatized with dialkyl amino benzaldehyde to form a derivatized poly(vinyl alcohol) comprising an acetal group, wherein the alkyl group comprises 1 to 6 carbon atoms. The reaction can occur at multiple sites in the latex, resulting in a distribution of reactive sites in latex polymers, which may vary from 0 to 1 to 2 and higher. The stoichiometry of the reaction in Step C is preferably controlled so that one acetal function per poly(vinyl alcohol) chain has the highest probability. A Poisson distribution suggests the following distribution.

| Attachments per chain | Fraction of total |
|-----------------------|-------------------|
| 0                     | $1/e = 0.368$     |
| 1                     | $1/e = 0.368$     |
| 2                     | $1/2e = 0.184$    |
| $>2$                  | $1-2.5/e = 0.08$  |

In one embodiment of Step (B) above, the formation of the linking-group-containing shell polymer can be represented, for example, by the following reaction:



One amine function per poly(vinyl alcohol) chain is desired. Of course, the present invention is not limited to poly(vinyl alcohol) or the particular linking agent exemplified in this reaction.

In one embodiment, the overall reaction scheme for making a cationic core-shell polymeric particle can be represented, for example, as follows:





In a preferred embodiment, insoluble cationic core-shell polymeric particles are formed, each comprising a core and shell, a core comprising cationic core polymer having at least 10 mole percent of a cationic mordant monomeric unit and a shell comprising hydrophilic shell polymer, wherein the shell is at least 10% by weight of the core, wherein the shell polymer is linked to the core polymer through a linking group between the core polymer and shell polymer comprising an amine group relatively closer to the core and an acetal group relatively closer to the shell.

The amount of the water-insoluble core-shell particles in the image-receiving layer should be high enough so that the images printed on the recording element will have a sufficiently high density, but low enough so that the interconnected pore structure formed by the aggregates is not unduly filled or blocked, which might cause coalescence. The mordant polymer described above may be used in any amount effective for the intended purpose. In general, good results have been obtained when the mordant polymer is present in

an amount of about 5% to about 25% by weight of the top layer, preferably about 10%. In a preferred embodiment of the invention, the inorganic particles are present in an amount from about 10 to about 95 weight % of the image-recording layer, and the water-insoluble core-shell particles are present in an amount of from about 5 to about 30 weight %.

The addition of the mordant to the overcoat layer does not degrade or unduly degrade other performance features such as dry time, coalescence, bleeding, and adhesion of the layers, 10 water fastness, when printed with a variety of inkjet inks.

According to the invention, organic or inorganic particles are present in the amount of greater than fifty percent by weight, preferably between 60 and 95 percent by weight, of the image-receiving layer. The weight ratio of the insoluble 15 cationic core-shell polymeric particles to the total amount of inorganic/organic particles in the image-receiving layer is preferably 1:2 to 1:20, preferably 1:3 to 1:10.

In a preferred embodiment of the invention, the ink-retaining 20 layer is a continuous, co-extensive porous layer that contains organic or inorganic particles. Examples of organic particles which may be used include core/shell particles such as those disclosed in U.S. Pat. No. 6,492,006, and homogeneous particles such as those disclosed in U.S. Pat. No. 6,475,602, the disclosures of which are hereby incorporated by reference. Examples of organic particles that may be used include 25 acrylic resins, styrenic resins, cellulose derivatives, polyvinyl resins, ethylene-allyl copolymers and polycondensation polymers such as polyesters.

Examples of inorganic particles useful in the invention 30 include alumina, hydrated alumina such as boehmite, silica, titanium dioxide, zirconium dioxide, clay, calcium carbonate, inorganic silicates or barium sulfate. The particles may be porous or nonporous, colloidal or aggregated. In one embodiment of the invention, the inorganic particles are metallic 35 oxides, preferably fumed. Preferred examples of fumed metallic oxides that may be used include silica and alumina fumed oxides. Fumed oxides are available in dry form or as dispersions of the aggregates.

Many types of inorganic particles are manufactured by 40 various methods and commercially available for use in an image-receiving layer, which can provide porosity in the image-receiving layer in order to obtain very fast ink drying. The pores formed between the inorganic particles must be sufficiently large and interconnected so that the printing ink 45 passes quickly through the layer and away from the outer surface to give the impression of fast drying. At the same time, the particles must be arranged in such a way so that the pores formed between them are sufficiently small so that they do not scatter visible light.

In one embodiment of the invention, the image-receiving 50 layer comprises inorganic particles in the form of aggregated particles. The aggregates are comprised of smaller primary particles about 7 to about 40 nm in diameter, and are aggregated up to about 500 nm in diameter, preferably having a mean aggregate particle size of from about 50 nm to about 200 nm.

Examples of colloidal particles useful in the invention include alumina, hydrated alumina such as boehmite, silica, titanium dioxide, zirconium dioxide, clay, calcium carbonate, 60 inorganic silicates, and barium sulfate. Examples of optional organic particles useful in the invention are disclosed and claimed in U.S. Pat. Nos. 6,364,477; 6,492,006; 6,380,280; 6,475,602; 6,376,599; and 6,541,103; the disclosures of which are hereby incorporated by reference. In a preferred embodiment of the invention, the colloidal particles are silica or hydrated alumina such as boehmite. In a preferred embodiment of the invention, the colloidal particles may be in the

form of particles having a mean particle size in a range from about 20 nm to about 500 nm.

In a preferred embodiment of the invention, the image-receiving layer also contains a polymeric binder in an amount insufficient to alter the porosity of the porous receiving layer. In another preferred embodiment, the polymeric binder is a hydrophilic polymer such as poly(vinyl alcohol), poly(vinyl pyrrolidone), gelatin, cellulose ethers, poly(oxazolines), poly(vinylacetamides), partially hydrolyzed poly(vinyl acetate/vinyl alcohol), poly(acrylic acid), poly(acrylamide), poly(alkylene oxide), sulfonated or phosphated polyesters and polystyrenes, casein, zein, albumin, chitin, chitosan, dextran, pectin, collagen derivatives, collodian, agar-agar, arrowroot, guar, carrageenan, tragacanth, xanthan, rhamsan and the like. In still another preferred embodiment of the invention, the hydrophilic polymer is poly(vinyl alcohol), hydroxypropyl cellulose, hydroxypropyl methyl cellulose, hydroxyethyl cellulose, gelatin, or a poly(alkylene oxide). In yet still another preferred embodiment, the hydrophilic binder is poly(vinyl alcohol). The polymeric binder should be chosen so that it is compatible with the aforementioned particles.

The amount of binder used should be sufficient to impart cohesive strength to the inkjet recording element, but should also be minimized so that the interconnected pore structure formed by the aggregates is not filled in by the binder. In a preferred embodiment of the invention, the binder is present in an amount of from about 5 to about 20 weight %.

The thickness of the image-receiving layer may range from about 0.5 to about 50  $\mu\text{m}$ , preferably from about 1 to about 40  $\mu\text{m}$ . The coating thickness required is determined through the need for the coating to act as a sump for absorption of ink solvent and the need to hold the ink near the coating surface.

In a preferred embodiment, the recording element also contains a base layer having at least about 50 percent by weight of inorganic particles, preferably at least 70 percent by weight. The base layer is coated between the support and the image-receiving layer. In another preferred embodiment, the inorganic particles in the base layer comprise calcium carbonate, magnesium carbonate, barium sulfate, silica, alumina, boehmite hydrated alumina, clay or titanium oxide. In another preferred embodiment, the inorganic particles in the base layer have an anionic surface charge. In yet another preferred embodiment, the inorganic particles in the base layer have a mean particle size of from about 100 nm to about 5  $\mu\text{m}$ .

In still another preferred embodiment, the base layer contains a binder such as a polymeric material and/or a latex material, such as poly(vinyl alcohol) and/or styrene-butadiene latex. In still another preferred embodiment, the binder in the base layer is present in an amount of from about 5 to about 20 weight %. In still another preferred embodiment, the thickness of the base layer may range from about 5  $\mu\text{m}$  to about 50  $\mu\text{m}$ , preferably from about 20 to about 40  $\mu\text{m}$ .

After coating, the inkjet recording element may be subject to calendering or supercalendering to enhance surface smoothness. In a preferred embodiment of the invention, the inkjet recording element is subject to hot, soft-nip calendering at a temperature of about 65° C. and pressure of 14000 kg/m at a speed of from about 0.15 m/s to about 0.3 m/s.

The support for the inkjet recording element used in the invention can be any of those usually used for inkjet receivers, such as resin-coated paper, paper, polyesters, or microporous materials such as polyethylene polymer-containing material sold by PPG Industries, Inc., Pittsburgh, Pa. under the trade name of TESLIN, TYVEK synthetic paper (DuPont Corp.), and OPPALYTE films (Mobil Chemical Co.) and other composite films listed in U.S. Pat. No. 5,244,861. Opaque sup-

ports include plain paper, coated paper, synthetic paper, photographic paper support, melt-extrusion-coated paper, and laminated paper, such as biaxially oriented support laminates. Biaxially oriented support laminates are described in U.S. Pat. Nos. 5,853,965; 5,866,282; 5,874,205; 5,888,643; 5,888,681; 5,888,683; and 5,888,714, the disclosures of which are hereby incorporated by reference. These biaxially oriented supports include a paper base and a biaxially oriented polyolefin sheet, typically polypropylene, laminated to one or both sides of the paper base. Transparent supports include glass, cellulose derivatives, e.g., a cellulose ester, cellulose triacetate, cellulose diacetate, cellulose acetate propionate, cellulose acetate butyrate; polyesters, such as poly(ethylene terephthalate), poly(ethylene naphthalate), poly(1,4-cyclohexanedimethylene terephthalate), poly(butylene terephthalate), and copolymers thereof; polyimides; polyamides; polycarbonates; polystyrene; polyolefins, such as polyethylene or polypropylene; polysulfones; polyacrylates; polyetherimides; and mixtures thereof. The papers listed above include a broad range of papers, from high end papers, such as photographic paper to low end papers, such as newsprint. In a preferred embodiment, polyethylene-coated paper is employed.

The support used in the invention may have a thickness of from about 50 to about 500  $\mu\text{m}$ , preferably from about 75 to 300  $\mu\text{m}$ . Antioxidants, antistatic agents, plasticizers and other known additives may be incorporated into the support, if desired.

In order to improve the adhesion of the ink-receiving layer to the support, the surface of the support may be subjected to a corona-discharge treatment prior to applying the image-receiving layer.

Coating compositions employed in the invention may be applied by any number of well known techniques, including dip-coating, wound-wire rod coating, doctor blade coating, rod coating, air knife coating, gravure and reverse-roll coating, slide coating, bead coating, extrusion coating, curtain coating and the like. Known coating and drying methods are described in further detail in Research Disclosure No. 308119, published Dec. 1989, pages 1007 to 1008. Slide coating is preferred, in which the base layers and overcoat may be simultaneously applied. After coating, the layers are generally dried by simple evaporation, which may be accelerated by known techniques such as convection heating.

In order to impart mechanical durability to an inkjet recording element, crosslinkers, which act upon the binder discussed above, may be added in small quantities. Such an additive improves the cohesive strength of the layer. Crosslinkers such as carbodiimides, polyfunctional aziridines, aldehydes, isocyanates, epoxides, boric acid, polyvalent metal cations, and the like may all be used.

To improve colorant fade, UV absorbers, radical quenchers or antioxidants may also be added to the image-receiving layer, as is well known in the art. Other additives include pH modifiers, adhesion promoters, rheology modifiers, surfactants, biocides, lubricants, dyes, optical brighteners, matte agents, antistatic agents, etc. In order to obtain adequate coatability, additives known to those familiar with such art, such as surfactants, defoamers, alcohol and the like may be used. A common level for coating aids is 0.01 to 0.30% active coating aid based on the total solution weight. These coating aids can be nonionic, anionic, cationic or amphoteric. Specific examples are described in MCCUTCHEON's Volume 1: Emulsifiers and Detergents, 1995, North American Edition.

The coating composition can be coated either from water or organic solvents, however water is preferred. The total solids content should be selected to yield a useful coating thickness

in the most economical way, and for particulate coating formulations, solids contents from 10-40% are typical.

Inkjet inks used to image the recording elements of the present invention are well known in the art. The ink compositions used in inkjet printing typically are liquid compositions comprising a solvent or carrier liquid, dyes or pigments, humectants, organic solvents, detergents, thickeners, preservatives, and the like. The solvent or carrier liquid can be solely water or can be water mixed with other water-miscible solvents such as polyhydric alcohols. Inks in which organic materials, such as polyhydric alcohols, are the predominant carrier or solvent liquid may also be used. Particularly useful are mixed solvents of water and polyhydric alcohols. The dyes used in such compositions are typically water-soluble direct or acid type dyes. Such liquid compositions have been described extensively in the prior art including, for example, U.S. Pat. Nos. 4,381,946; 4,239,543; and 4,781,758, the disclosures of which are hereby incorporated by reference.

Although the recording elements disclosed herein have been referred to primarily as being useful for inkjet printers, they also can be used as recording media for pen plotter assemblies. Pen plotters operate by writing directly on the surface of a recording medium using a pen consisting of a bundle of capillary tubes in contact with an ink reservoir.

Emulsion polymerization is a heterogeneous, free-radical-initiated chain polymerization in which a monomer or a mixture of monomers is polymerized in the presence of an aqueous solution of a surfactant to form a latex, which is a colloidal dispersion of polymer particles in an aqueous medium. Emulsion polymerization is well known in the art and is described, for example, in F. A. Bovey, *Emulsion Polymerization*, issued by Interscience Publishers Inc. New York, 1955; and P. A. Lovell and M. El-Aasser, *Emulsion Polymerization and Emulsion Polymers*, issued by John Wiley and Sons, Chichester, 1997.

The basic components of an emulsion polymerization include water, initiators, surfactants, monomers, and optional additives and addenda such as chain transfer agents, biocides, colorants, antioxidants, buffers, and rheological modifiers. Emulsion polymerizations can be carried out via a batch process, in which all of the components are present at the beginning of the reaction, a semibatch process, in which one or more of the ingredients is added continuously, or a continuous process, in which the ingredients are fed into a stirred tank or more than one tank in series and the product latex is continuously removed. Intermittent or "shot" addition of monomers may also be used.

The monomers useful in an emulsion polymerization will include 75-100% of water-immiscible monomers and 0-25% of water-miscible monomers. Water-immiscible monomers useful in this embodiment of this invention include methacrylic acid esters, such as methyl methacrylate, ethyl methacrylate, isobutyl methacrylate, 2-ethylhexyl methacrylate, benzyl methacrylate, phenoxyethyl methacrylate, cyclohexyl methacrylate and glycidyl methacrylate, acrylate esters such as methyl acrylate, ethyl acrylate, isobutyl acrylate, 2-ethylhexyl acrylate, benzyl methacrylate, phenoxyethyl acrylate, cyclohexyl acrylate, and glycidyl acrylate, styrenes such as styrene,  $\alpha$ -methylstyrene, 3- and 4-chloromethylstyrene, halogen-substituted styrenes, and alkyl-substituted styrenes, vinyl halides and vinylidene halides, N-alkylated acrylamides and methacrylamides, vinyl esters such as vinyl acetate and vinyl benzoate, vinyl ether, allyl alcohol and its ethers and esters, and unsaturated ketones and aldehydes such as acrolein and methyl vinyl ketone, isoprene, butadiene and cyanoacrylate esters. In addition, any of the acrylate, sty-

renics, and crosslinking monomers listed previously in this document that are water-insoluble can be used.

Water-miscible monomers are useful in the present invention. Such monomers include the charged monomers that contain ionic groups as discussed previously. Other useful monomers include monomers containing hydrophilic, non-ionic units such as poly(ethylene oxide) segments, carbohydrates, amines, amides, alcohols, polyols, nitrogen-containing heterocycles, and oligopeptides. Examples of nonionic, water-miscible monomers include, but are not limited to poly(ethylene oxide) acrylate and methacrylate esters, vinylpyridines, hydroxyethyl acrylate, glycerol acrylate and methacrylate esters, (meth)acrylamide, and N-vinylpyrrolidone.

Initiators which are useful in this embodiment of this invention include both water-soluble and water-insoluble initiators, although the former class is preferred. These include, but are not restricted to azo compounds, such as 2,2'-azobis(4-methoxy-2,4-dimethylvaleronitrile), (1-phenylethyl)azodiphenylmethane, 2,2'-azobisisobutyronitrile (AIBN), 1,1'-azobis(1-cyclohexanedicarbonitrile), 4,4'-azobis(4-cyanovaleric acid), and 2,2'-azobis(2-amidinopropane)dihydrochloride, organic peroxides, organic hydroperoxides, peresters, and peracids such as benzoyl peroxide, lauryl peroxide, capryl peroxide, acetyl peroxide, t-butyl hydroperoxide, t-butyl perbenzoate, cumyl hydroperoxide, peracetic acid, 2,5-dimethyl-2,5-di(peroxybenzoate), and p-chlorobenzoyl peroxide, persulfate salts such as potassium, sodium and ammonium persulfate, disulfides, tetrazenes, and redox initiator systems such as  $H_2O_2/Fe^{2+}$ , persulfate/bisulfite, oxalic acid/Mn<sup>3+</sup>, thiourea/Fe<sup>3+</sup>, and benzoyl peroxide/dimethylaniline. Preferred initiators for this embodiment of this invention include persulfate salts (optionally used in combination with bisulfite), 4,4'-azobis(4-cyanovaleric acid), and 2,2'-azobis(2-amidinopropane)dihydrochloride.

Emulsion polymerizations additionally require a stabilizer compound that is used to impart colloidal stability to the resultant particles. These compounds may be surfactants or protective colloids, which are oligomeric or macromolecular amphiphiles. There exists a tremendous number of other known surfactant compounds. Good reference sources for surfactants are the *Surfactant Handbook* (GPO: Washington, D. C., 1971) and *McCUTCHEON'S Emulsifiers and Detergents* (Manufacturing Confectioner Publishing Company: Glen Rock, 1992). Surfactants can be anionic, cationic, zwitterionic, neutral, low molecular weight, macromolecular, synthetic, or extracted or derived from natural sources. Some examples include, but are not necessarily limited to: sodium dodecylsulfate, sodium dodecylbenzenesulfonate, sulfosuccinate esters, such as those sold under the AEROSOL trade name, fluorosurfactants, such as those sold under the ZONYL and FLUORAD trade names, ethoxylated alkylphenols, such as TRITON X-100 and TRITON X-705, ethoxylated alkylphenol sulfates, such as RHODAPEX CO-436, phosphate ester surfactants such as GAFAC RE-90, hexadecyltrimethylammonium bromide, polyoxyethylenated long-chain amines and their quaternized derivatives, ethoxylated silicones, alkanolamine condensates, polyethylene oxide-co-polypropylene oxide block copolymers, such as those sold under the PLURONIC and TECTRONIC trade names, N-alkylbetaines, N-alkyl amine oxides, and fluorocarbon-poly(ethylene oxide) block surfactants, such as FLUORAD FC-430. Protective colloids useful in this invention include, but are not necessarily limited to: poly(ethylene oxide), hydroxyethyl cellulose, poly(vinyl alcohol), poly(vinyl pyrrolidone), polyacrylamides, polymethacrylamides, sulfonated polystyrenes, alginates, carboxy methyl cellulose, polymers and copolymers of dimethylaminoethyl methacry-

## 17

late, water soluble complex resinous amine condensation products of ethylene oxide, urea and formaldehyde, polyethyleneimine, casein, gelatin, albumin, gluten and xanthan gum.

Polymeric particles can be prepared by suspension, mini-emulsion or micro-suspension polymerizations. The terms "mini-emulsion" and "micro-suspension" will be used interchangeably throughout this document. "Suspension polymerization" refers to a process in which a polymerizable liquid is dispersed as droplets in a continuous aqueous medium and polymerized under continuous agitation. Any of the initiators described above for emulsion polymerization can be used in suspension, and mini-emulsion/micro-suspension polymerizations. Preferably, organic-soluble initiators will be used. Normally, this process is carried out in the presence of a "granulating agent," such as a lyophilic polymer (starch, natural gums, polyvinyl alcohol or the like) or an insoluble fine powder such as calcium phosphate. These granulating agents help to obtain a dispersion of droplets of the polymerizable liquid but do not provide sufficient stabilization of the dispersion so that the dispersed droplets are stable in the absence of agitation. Therefore, in this method, it is necessary to carry out the polymerization under continuous high-energy mechanical agitation, since otherwise extensive coalescence of the droplets will occur, with separation of a bulk phase of the water immiscible, polymerizable material or the formation of large amounts of coagulum. Because this process depends on the details of the shear field in the reactor, and on the changing viscosity of the polymerizing dispersed phase, it is difficult to control reproducibly, is not readily scalable, and gives broad particle size distributions. Suspension polymerization is further described in U.S. Pat. Nos. 5,889,285; 5,274,057; 4,601,968; 4,592,990; R. Arshady "Suspension, emulsion, and dispersion polymerization: A methodological survey" *Colloid Polym. Sci.* 270: 717-732 (1992); and H. G. Yuan, G. Kalfas, W. H. Ray *JMS-Rev. Macromol. Chem. Phys.* C31 (2-3): 215 (1991).

The term mini-emulsion or micro-suspension polymerization also refers to a process in which the water-immiscible polymerizable liquid is dispersed in an aqueous medium. In this process, as in suspension polymerization, the water insoluble monomer is dispersed in the presence of a dispersion stabilizer or granulating agent to the desired size by using a mechanical shearing device such as an agitator, a high pressure homogenizer, colloid mill, ultrasonic horn or the like. In contrast to simple suspension polymerization, however, in mini-emulsion or micro-suspension polymerization, the polymerization can then be carried out with no or minimal stirring (only enough to prevent creaming and provide good thermal transfer). Various dispersion stabilizers or granulating agents are well known in the art (for example, surfactants such as sodium dodecyl sulfate or sodium dioctylsulfosuccinate, and hydrophilic polymers, for example polyvinyl alcohol, gelatin, methyl cellulose, methylhydroxypropyl cellulose, ethyl cellulose, sodium salt of carboxymethyl cellulose, polyacrylic acid and salts thereof, starch, gum, alginic acid salts, zein, casein). In some cases, granulating agents useful for suspension polymerization are also useful for microsuspension polymerization. Which process occurs is a function of the nature of the oil phase, that is, whether the dispersion is stable in the absence of mechanical agitation or whether it will coalesce before or during the polymerization process. Suspension polymerization is used to provide easily filterable polymer products, but these products are generally of ill-defined particle size and size distribution, usually of between 50-1000 micrometers. Mini-emulsion and micro-suspension polymerization can be used to provide products with mean

## 18

particle sizes less than 20 micrometers. Mini-emulsion and micro-suspension polymerization are described in U.S. Pat. Nos. 5,858,634; 5,492,960; J. Ugelstad, M. S. El-Aasser, and J. W. Vanderhoff, *J. Polym. Sci. Polym. Lett. Ed.*, 11, 503 (1973); and Sudol, E. D. and El-Aasser, M. in *Emulsion Polymerization and Emulsion Polymers*, Lovell, P. A. and El-Aaser, M. Eds., John Wiley and Sons Ltd., New York, 1997; p. 699-721.

The water dispersible polymer particle may be made by a dispersion polymerization. Dispersion polymerization is a technique in which a monomer or a monomer mixture is polymerized in a solvent or solvent mixture that is a solvent for the monomer and a non-solvent for the polymer. A stabilizer compound is used to produce a colloidally stable dispersion. A discussion of this type of polymerization is given by J. L. Cawse in *Emulsion Polymerization and Emulsion Polymers*, Lovell, P. A. and El-Aaser, M. Eds., John Wiley and Sons Ltd., New York, 1997; p. 699-721. It is known in the art that steric (nonionic) stabilizers are especially important in this type of polymerization.

The water dispersible polymer particle may be made by solvent evaporation. This involves first forming a solution of a polymer in a solvent that is immiscible with water (along with any required addenda), and then suspending the polymer-solvent solution in water containing a hydrophobically capped oligomeric acrylamide dispersant. The resulting suspension is subjected to high shear action to reduce the size of the polymer-solvent droplets. The shearing action is optionally removed and the polymer-solvent droplets coalesce to the extent allowed by the dispersant to form coalesced polymer-solvent droplets. The solvent is removed from the drops to form solidified polymer particles that are then optionally isolated from the suspension by filtration or other suitable means.

Any suitable solvent that will dissolve the polymer and which is also immiscible with water may be used, such as for example, chloromethane, dichloromethane, ethyl acetate, n-propyl acetate, iso-propyl acetate, vinyl chloride, methyl ethyl ketone (MEK), trichloromethane, carbon tetrachloride, ethylene chloride, trichloroethane, toluene, xylene, cyclohexanone, 2-nitropropane and the like. Preferred are n-propyl acetate, iso-propyl acetate, ethyl acetate and methylene chloride. Particularly preferred is n-propyl acetate or ethyl acetate.

## EXAMPLES

Preparation of the Core Polymer Intermediate 1  
(PI-1)

A mixture of monomers consisting of 292 g vinyl benzyl chloride (mixed isomers, Dow Chemical) and 34.2 g divinyl benzene (55% assay, mixed isomers Dow Chemical) were emulsified in 296 g demineralized water and 42 g RHODAON UB (29% sodium lauryl sulfate, Rhodia Inc.) and 0.57 g sodium metabisulfite. The emulsion was maintained by continual stirring.

The polymerization reaction was carried out as follows. Demineralized water (990 g) and 13.9 g Rhodapon UB were added to a 2 L reactor previously flushed with nitrogen and heated to 60° C. When the reactor reached 60° C., 0.16 g sodium metabisulfite and 2.2 g sodium persulfate were added. The monomer emulsion was then added continuously over a

19

four hour time period. The reactor was held at 60° C. for an additional four hours and then cooled to 25° C. The particle size of the latex was 60 nm.

Preparation of the Core Polymer Intermediate 2  
(PI-2)

A mixture of monomers consisting of 292 g vinyl benzyl chloride (mixed isomers, Dow Chemical) and 34.2 g divinyl benzene (55% assay, mixed isomers Dow Chemical) was emulsified in 296 g demineralized water and 16.7 g RHODAPON UB (29% sodium lauryl sulfate, Rhodia Inc.) and 0.57 g sodium metabisulfite. The emulsion was maintained by continual stirring.

Polymerization of the monomer mixture was carried out as follows. Demineralized water (990 g) and 6.6 g Rhodapon UB were added to a 2 L reactor previously flushed with nitrogen and heated to 60° C. When the reactor reached 60° C., 0.16 g sodium metabisulfite and 2.2 g sodium persulfate were added. The monomer emulsion was then added continuously over a four hour time period. The reactor was held at 60° C. for an additional four hours and then cooled to 25° C. The particle size of the latex was 110 nm, which was larger than that of the core polymer intermediate PI-1, as a result of less surfactant being employed in the emulsion polymerization

Preparation of Comparative Mordant (Non-Core-Shell) Polymer Particle 1 (CP-1)

Preparation of a comparative mordant polymer particle, without a shell, was carried out by quaternization of core polymer PI-1, in which 500 g of PI-1 were quaternized by adding 111 g of trimethylamine (25% aq., Aldrich). During the trimethylamine addition it was necessary to increase the stirring as the reaction mixture thickened and then reduce it again when the mixture thinned. After the quaternization was complete, residual trimethyl amine was removed by raising the pH of the mixture to 12 and distilling the mixture under vacuum at approximately 65° C. for three hours.

The resulting sample was 12.4% solids as determined by gravimetric analysis, had less than 1 µg/g residual trimethylamine as determined by ion chromatography, had median particle size of 91 nm as determined by UPA, had a pH of 3.6, and was determined by silver nitrate titration to be 80.6 weight % vinylbenzyltrimethylammonium chloride. The zeta potential at pH 4 was 36.2 mV, at pH 7 was 36.4 mV, at pH 10 was 30.4 mV.

The zeta potential of a dispersed particle is defined as the electrostatic potential generated at the junction of the rigidly attached Stern layer and the weakly associated diffuse layer and is stated in the units of millivolts.

The zeta potential of a particle can be calculated, knowing the electrophoretic mobility of the sample, by Henry's Equation:

$$U_e = \frac{2\epsilon\zeta f(ka)}{3\eta}$$

Where  $U_e$  is the electrophoretic mobility,  $\epsilon$  is the dielectric constant of the sample,  $\zeta$  is the zeta potential,  $f(ka)$  is Henry's Function, and  $\eta$  is the viscosity of the solvent. Usually, electrophoretic analysis is made in aqueous media for which  $f(ka)$  takes the value 1.5. This value is used in the Smoluchowski approximation to yield:

$$\mu_e = \epsilon\zeta/\eta$$

20

Classically, if the absolute value of the zeta potential is greater than 30 mV the particles will repel each other during collisions due to thermal motion. If the absolute value of the zeta potential is less than 30 mV, the collisions will result in flocculation and destabilization.

The electrophoretic mobility for these samples was quantified using a Malvern Instruments ZETASIZER Nano ZS. The instrument utilizes Laser Doppler Velocimetry where an electrical field of known strength is applied across the sample, 10 through which a laser is then passed. The electrophoretic mobility of the colloid will dictate the velocity with which the charged particles move which will then induce a frequency shift in the incident laser beam. Using the Smoluchowski approximation for Henry's Function, the dielectric constant 15 of the sample, the viscosity of the solvent and the measured electrophoretic mobility, the zeta potential of the particles for the samples was calculated.

Preparation of Comparative Mordant (Non-Core-Shell) Polymer Particle 2 (CP-2).

A comparative mordant polymer particle, without a shell was carried out by quaternization of core polymer PI-1, in which 500 g of CPI-2 were quaternized by adding 111 g of trimethylamine (25% aq., Aldrich). During the trimethylamine addition it was necessary to increase the stirring as the reaction mixture thickened and then reduce it again when the mixture thinned.

After the quaternization was complete, residual trimethyl amine was removed by raising the pH of the mixture to 12 and 30 distilling the mixture under vacuum at approximately 65° C. for three hours.

The resulting sample was 13.1% solids as determined by 35 gravimetric analysis, had less than 1 µg/g residual trimethylamine as determined by ion chromatography, had median particle size of 166 nm, larger than CP-1, as determined by UPA, had a pH of 2.7, and was determined by silver nitrate titration to be 81.0 weight % vinylbenzyltrimethylammonium chloride. The zeta potential at pH 4 was 33.9 mV, at pH 7 was 35.2 mV, and at pH 10 it was 24 mV.

Preparation of Core-Shell Polymer Particle 1 (PE-1)

A mixture of monomers consisting of 292 g vinyl benzyl chloride (mixed isomers, Dow Chemical) and 34.2 g divinyl benzene (55% assay, mixed isomers Dow Chemical) was emulsified in 296 g demineralized water and 42 g RHODAPON UB (29% sodium lauryl sulfate, Rhodia Inc.) and 0.57 g sodium metabisulfite. The emulsion was maintained by continual stirring.

The polymerization reaction was carried out by adding 990 50 g demineralized water, 13.9 g RHODAPON UB, and 200 g of CELVOL 203 (88% hydrolysis poly(vinyl alcohol), Celanese Inc.) to a 2 L reactor previously flushed with nitrogen, heated to 85° C., held for one hour to dissolve the polyvinylalcohol, and then cooled to 60° C. When the reactor reached 60° C., 55 0.16 g sodium metabisulfite and 2.2 g sodium persulfate were added. The monomer emulsion was then added continuously over a four hour time period. The reactor was held at 60° C. for an additional four hours and then cooled to 25° C.

The latex was quaternized by adding 380 g of trimethylamine (25% aq., Aldrich). During the trimethylamine addition it was necessary to increase the stirring as the reaction mixture thickened and then reduce it again when the mixture thinned.

After the quaternization was complete, residual trimethyl amine was removed by raising the pH of the mixture to 12 and 65 distilling the mixture under vacuum at approximately 65° C. for three hours.

The following Table 1 shows a comparison of core-shell particle PE-1 with comparative particle CP-1. Evidence for a nonionic shell around a cationic core include the observed increase in particle size and the reduction in zeta potential that indicates a shielding of the cationic core polymer. The weight percent quaternary ammonium salt analysis is a measure of the cationic content of the particle, and is used to normalize the mordant concentration in coatings.

TABLE 1

| Example          | Median Particle Size $\mu\text{m}$ | Wt % Quaternary Ammonium Salt | Zeta Potential |         |          |
|------------------|------------------------------------|-------------------------------|----------------|---------|----------|
|                  |                                    |                               | at pH 4        | at pH 7 | at pH 10 |
| Comparative CP-1 | 0.091                              | 80.6                          | 36.2           | 36.4    | 30.4     |
| Core-Shell-PE-1  | 0.101                              | 55.6                          | 6.7            | 3.9     | 3.8      |

#### Preparation of Linking-Group-Containing Shell Polymer 1 (SP-1)

A linking-group-containing shell polymer was prepared by dissolving 200 g of CELVOL 203 (88% hydrolyzed polyvinyl alcohol, estimated number average molecular weight 13,200, 0.015 moles, Celanese Inc.) in 800 g of water by heating to 90° C. and holding for one hour. The mixture was cooled to 60° C. 2.26 g (0.015 moles) of 4-dimethylaminobenzaldehyde and 6 mL of concentrated HCl were added to the solution and allowed to react overnight.

#### Preparation of Linking-Group-Containing Shell Polymer 2 (SP-2)

A linking-group-containing shell polymer was prepared by dissolving 200 g of Nippon Gohsei NK-05 (73% hydrolyzed, estimated number average molecular weight 15,400, 0.013 moles) in 800 g of demineralized water, by heating to 70° C. and holding for one hour. The mixture was then cooled to 60° C. and 2.64 g (0.0175 moles) of 4-dimethylaminobenzaldehyde and 6 mL of concentrated HCl were added to the solution and allowed to react overnight.

#### Preparation of Linking-Group-Containing Shell Polymer 3 (SP-3)

A linking-group-containing shell polymer was prepared by dissolving 300 g of CELVOL 103 were dissolved in 1200 g of demineralized water by heating to 95° C. and holding for one hour. The mixture was then cooled to 60° C. and 3.39 g of 4-dimethylaminobenzaldehyde and 9 mL of concentrated HCl were added to the solution and allowed to react overnight. Table 2 shows the characterization of the shell polymers by NMR. These data indicate that the reaction of the aldehyde with the polyvinyl alcohol is nearly quantitative, with a minimum of 88% of the aldehyde being converted to acetal. Additionally, the mole percent acetal data indicate

that, on average, there is approximately one acetal function per polyvinyl alcohol molecule.

TABLE 2

| 5  | Shell Polymer | Mole % vinyl alcohol | Mole % Acetate | Unincorporated Aldehyde % of Total Aldehyde |                     |
|----|---------------|----------------------|----------------|---------------------------------------------|---------------------|
|    |               |                      |                | Mole % Acetal                               | % of Total Aldehyde |
| 10 | SP-1          | 89                   | 11             | 0.34                                        | 2                   |
|    | SP-2          | 75                   | 24             | 0.46                                        | 5                   |
|    | SP-3          | 99                   | 1.1            | 0.30                                        | 12                  |

The results in Table 2 show a high yield of shell polymer with one or more acetal linking groups (1 to 2 linkages per poly(vinyl alcohol) polymer on average, as calculated based on NMR analysis.

The following Examples of core-shell particles according to the present examples show the effect of differing amounts of shell polymer relative to the same core polymer.

#### Preparation of Core-Shell Particle 2 (PE-2)

Another core-shell polymer, according to the present invention, was prepared by combining 300 g of SP-1 with 600 g of demineralized water and adjusting the pH to 10 with sodium hydroxide. The mixture was combined with 100 grams of CPI-2 and stirred for 30 minutes. Then, 22.14 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 3 (PE-3)

Another core-shell polymer, according to the present invention, was prepared by combining 300 g of SP-1 with 500 g of demineralized water and adjusting the pH to 10 with sodium hydroxide. The mixture was combined with 200 g of CPI-2 and stirred for 30 minutes. 44.28 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 4 (PE-4)

Another core-shell polymer, according to the present invention, was prepared by combining 200 g of SP-1 with 533 g of demineralized water and adjusting the pH to 10 with sodium hydroxide. The mixture was combined with 267 g of CPI-2 and stirred for 30 minutes. 59.1 g of trimethylamine (25% aq.) were added and allowed to stir for one hour. After one hour, the pH was raised to 12 and the mixture was vacuum distilled for 3 hours to remove residual trimethylamine.

Table 3 below shows a comparison of preparative examples PE-2, PE-3, and PE-4 representing a cationic core-shell particle with comparative example CE-2 representing a cationic particle.

TABLE 3

| Cationic Particle Example | Weight Ratio of Shell to Core | Median Particle Size $\mu\text{m}$ | Wt % Quaternary Ammonium Salt | Zeta Potential at pH 4 | Zeta Potential at pH 7 | Zeta Potential at pH 10 |
|---------------------------|-------------------------------|------------------------------------|-------------------------------|------------------------|------------------------|-------------------------|
| Comparative CE-2          | 0:1                           | 0.166                              | 81                            | 33.9                   | 35.2                   | 24                      |
| Example PE-2              | 2.8:1                         | 0.282                              | 29.2                          | 5.5                    | 7.8                    | 4.8                     |
| Example PE-3              | 2:1                           | 0.247                              | 40.4                          | 8.4                    | 9.3                    | 7.3                     |

TABLE 3-continued

| Cationic Particle Example | Weight Ratio of Shell to Core | Median Particle Size $\mu\text{m}$ | Wt % Quaternary Ammonium Salt | Zeta Potential at pH 4 | Zeta Potential at pH 7 | Zeta Potential at pH 10 |
|---------------------------|-------------------------------|------------------------------------|-------------------------------|------------------------|------------------------|-------------------------|
| Example PE-4              | 1.5:1                         | 0.213                              | 53.9                          | 11.5                   | 13.5                   | 11.8                    |

The weight percent of quaternary ammonium salt, with respect to the total weight of the particles, was calculated using ionic chloride concentrations determined by silver nitrate titration. The ionic species was assumed to be vinyl benzyl trimethyl ammonium chloride. The zeta potentials were determined as described above. The zeta potential data show that the reduction in zeta potential is proportional to amount of shell polymer. The particle size results show that as the proportion of shell polymer in the particle increases so does the median particle size.

#### Preparation of Core-Shell Particle 5 (PE-5)

Another core-shell polymer, according to the present invention, was prepared by combining 600 g of SP-1 with 600 g of demineralized water and adjusting the pH to 10 with sodium hydroxide. The mixture was combined with 200 g of CPI-1 and stirred for 30 minutes. 44.3 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 6 (PE-6)

Another core-shell polymer, according to the present invention, was prepared by combining 400 g of SP-1 with 533 g of demineralized water and adjusting the pH to 10 with sodium hydroxide. The mixture was combined with 534 g of CPI-1 and stirred for 30 minutes. 118.2 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 7 (PE-7)

Another core-shell polymer, according to the present invention, was prepared by combining 600 g of SP-3 (a shell polymer other than SP-1) with 600 g of demineralized water and adjusting the pH to 10 with sodium hydroxide. The mixture was combined with 200 g of CPI-1 and stirred for 30

minutes. 44.3 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 8 (PE-8)

Another core-shell polymer, according to the present invention, was prepared by combining 350 g of SP-3 with 466 g of demineralized water and adjusting the pH to 10 with sodium hydroxide. The mixture was combined with 467 g of CPI-1 and stirred for 30 minutes. 100.8 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 9 (PE-9)

Another core-shell polymer, according to the present invention, was prepared by combining 600 g of SP-2 (a shell polymer other than SP-1 or SP-3) with 600 g of demineralized water and adjusting the pH to 10 with sodium hydroxide. The mixture was combined with 200 g of CPI-1 and stirred for 30 minutes. 44.3 g of trimethylamine (25% aq.) were added and allowed to stir for one hour. After one hour, the pH was raised to 12 and the mixture was vacuum distilled for 3 hours to remove residual trimethylamine.

#### Preparation of Core-Shell Particle 10 (PE-10)

Another core-shell polymer, according to the present invention, was prepared by combining 350 g of SP-2 with 466 g of demineralized water and adjusting the pH to 10 with sodium hydroxide. The mixture was combined with 467 g of CPI-1 and stirred for 30 minutes. 100.8 g of trimethylamine (25% aq.) were added and allowed to stir for one hour. After one hour, the pH was raised to 12 and the mixture was vacuum distilled for 3 hours to remove residual trimethylamine.

Table 4 below shows a comparison of Core-Shell Particles PE-5 to PE-10 with Comparative Example CE-1

TABLE 4

| Example | Weight Ratio of Shell to Core | Median Particle Size $\mu\text{m}$ | Wt % Quaternary Ammonium Salt | Zeta Potential at pH 4 | Zeta Potential at pH 7 | Zeta Potential at pH 10 |
|---------|-------------------------------|------------------------------------|-------------------------------|------------------------|------------------------|-------------------------|
| CE-1    | 0:1                           | None                               | 0.091                         | 80.6                   | 36.2                   | 36.4                    |
| PE-5    | 2.8:1                         | SP-1                               | 0.123                         | 28.8                   | 2.9                    | 0.6                     |
| PE-6    | 1.6:1                         | SP-1                               | 0.119                         | 51.9                   | 5.6                    | 2.5                     |
| PE-7    | 2.4:1                         | SP-3                               |                               | 33.3                   | 2.1                    | 0.2                     |
| PE-8    | 1.5:1                         | SP-3                               |                               | 55.3                   | 5.2                    | 1.8                     |
| PE-9    | 2.7:1                         | SP-2                               | 0.137                         | 30.2                   | 0.6                    | -0.5                    |
| PE-10   | 1.5:1                         | SP-2                               | 0.128                         | 52.4                   | 3.4                    | 1.3                     |

The results in Table 4 confirm that as the amount of shell polymer is increased the median particle size also increases. This is evidence that the shell polymer is reacting with the core to form a larger shelled particle. The zeta potential data shows that as the amount of shell polymer increases the zeta potential decreases, which is an indication of shielding of the cationic core by the nonionic shell.

## Comparative Example 1

## Coating Comparative Receiver Element CR-1

A multilayer inkjet receiver was prepared as follows. A coating composition for a base layer was prepared by mixing 0.335 dry g of COLLOID 211 sodium polyacrylate (Kemira Chemicals) as a 43% solution with 145 g of water. To the mixture was added 25.44 dry g of silica gel (IJ-624, Crosfield Ltd.) while stirring, 148.3 dry g of precipitated calcium carbonate (ALBAGLOSS-S, Specialty Minerals Inc.) as a 69% solution, 4.09 dry g of a polyvinyl alcohol (CELVOL 325, Air Products and Chemicals Inc.) as a 10% solution, an additional 22.89 dry g of silica gel (IJ-624, Crosfield Ltd.), and 25 dry g of styrene-butadiene latex (CP692NA, Dow Chemicals) as a 50% solution. The silica gel was added in two parts to avoid gelation.

Accordingly, the base layer coating composition was made up of the sodium polyacrylate, silica gel, precipitated calcium carbonate, polyvinyl alcohol, and styrene-butadiene latex in a weight ratio of 0.15:21.30:65.45:1.80:11.30 at 45% solids.

The base layer coating composition was rod-coated on a base paper, basis weight 179 g/m<sup>2</sup>, and dried by forced air. The thickness of the dry base coating was 30 µm and its weight was 32.3 g/m<sup>2</sup>.

A coating composition for the intermediate layer was prepared by combining hydrated alumina (CATAPAL 200, Sasol Corp.), poly(vinyl alcohol) (GOHSENOL GH-23, Nippon Gohsei Co.), CARTABOND GH (Clariant Corp.) glyoxal crosslinker and boric acid in a ratio of 95.38:4.25:0.25:0.13, to give an aqueous coating formulation of 33% solids by weight.

A coating composition for the upper layer was prepared by combining hydrated alumina (DISPAL 14N4-80, Condea Vista Co.), fumed alumina (Cab-O-SPERSE PG003, Cabot Corp.), polyvinyl alcohol (GOHSENOL GH-23, Nippon Gohsei Co.), comparative cationic mordant particles CE-1 as prepared above, CARTABOND GH glyoxal (Clariant Corp.) and boric acid in a ratio of 36.4:41.58:5.23:15.72:0.25:0.13 to give an aqueous coating formulation of 21% solids by weight. Surfactants ZONYL FSN (DuPont Co.) and OLIN 10G (Olin Corp.) were added in small amounts as coating aids.

The intermediate and upper layer coating compositions were bead coated on top of the base layer. The coating was then dried by forced air to yield a three-layer recording element. The thickness of the mid-layer was 35 µm or 37.7 g/m<sup>2</sup>. The thickness of the overcoat-layer was 2 µm or 2.15 g/m<sup>2</sup>. The coated material was calendered at a pressure of 700 pli, including two passes through the nip.

## Example 1

A multilayer inkjet receiver Element R-1, according to the present invention, comprising RPP core-shell polymer SC-1, was prepared the same way as element CR-1, except the polyvinyl alcohol and the cationic mordant were replaced with PE-1, where the cationic content was kept equivalent.

## Comparative Example 2

A multilayer inkjet receiver Comparative Element CR-2 was prepared the same way as element C-1, except the cationic mordant was replaced with CE-2.

## Comparative Example 3

A multilayer inkjet receiver Comparative Element CR-3 was prepared the same way as element C-1, except the cationic mordant was increased by 50%.

## Example 2

A multilayer inkjet receiver Element R-2, according to the present invention, was prepared the same way as element C-1, except the polyvinyl alcohol and cationic mordant were replaced with PE-2, where the cationic content was kept equivalent.

## Example 3

A multilayer inkjet receiver Element R-3, according to the present invention, was prepared the same way as element C-1, except the polyvinyl alcohol and cationic mordant were replaced with PE-3, where the cationic content was kept equivalent.

## Example 4

A multilayer inkjet receiver Element R-4, according to the present invention, was prepared the same way as element C-1, except the polyvinyl alcohol and cationic mordant were replaced with PE-4, where the cationic content was kept equivalent.

## Example 5

A multilayer inkjet receiver Element R-5, according to the present invention, was prepared the same way as element C-1, except the polyvinyl alcohol and cationic mordant were replaced with PE-5, where the cationic content was kept equivalent.

## Example 6

A multilayer inkjet receiver Element R-6, according to the present invention, was prepared the same way as element C-1, except the polyvinyl alcohol and cationic mordant were replaced with PE-5, where the cationic content was increased by 50%.

## Example 7

A multilayer inkjet receiver Element R-1, according to the present invention, was prepared the same way as element C-1, except the polyvinyl alcohol and cationic mordant were replaced with PE-6, where the cationic content was kept equivalent.

## Example 8

A multilayer inkjet receiver Element R-8, according to the present invention, was prepared the same way as element C-1, except the polyvinyl alcohol and cationic mordant were replaced with PE-6, where the cationic content was increased by 50%.

## Example 9

A multilayer inkjet receiver Element R-9, according to the present invention, was prepared the same way as element C-1, except the polyvinyl alcohol and cationic mordant were replaced with PE-7, where the cationic content was kept equivalent.

## Example 10

A multilayer inkjet receiver Element R-10, according to the present invention, was prepared the same way as element

C-1, except the polyvinyl alcohol and cationic mordant were replaced with PE-7, where the cationic content was increased by 50%.

## Example 11

A multilayer inkjet receiver Element R-1, according to the present invention, was prepared the same way as element C-1, except the polyvinyl alcohol and cationic mordant were replaced with PE-8, where the cationic content was kept equivalent.

## Example 12

A multilayer inkjet receiver Element R-12, according to the present invention, was prepared the same way as element C-1, except the polyvinyl alcohol and cationic mordant were replaced with PE-8, where the cationic content was increased by 50%.

## Example 13

A multilayer inkjet receiver Element R-13, according to the present invention, was prepared the same way as element C-1, except the polyvinyl alcohol and cationic mordant were replaced with PE-9, where the cationic content was kept equivalent.

## Example 14

A multilayer inkjet receiver Element R-14, according to the present invention, was prepared the same way as element C-1, except the polyvinyl alcohol and cationic mordant were replaced with PE-9, where the cationic content was increased by 50%.

## Example 15

A multilayer inkjet receiver Element R-14, according to the present invention, was prepared the same way as element

C-1, except the polyvinyl alcohol and cationic mordant were replaced with PE-10, where the cationic content was kept equivalent.

5

## Example 16

A multilayer inkjet receiver Element R-16, according to the present invention, was prepared the same way as element C-1, except the polyvinyl alcohol and cationic mordant were replaced with PE-10, where the cationic content was increased by 50%.

## Experimental Testing of Fade Density

Dye fade was evaluated by printing a test target of uniform density patches on test samples with a Hewlett Packard Model 6540 inkjet printer. After printing the densities were read with a SPCTROLINO Spectroscan T densitometer manufactured by Greystag Macbeth. The test samples were then placed into a 60 ppb ozone chamber and held there for seven days. After removal, the densities of the test strips were reread, and the percent fade at an optical density of 1.0 was interpolated from the fade data.

The results of testing of Comparative Elements C-1, C-2, and C-3 and Elements R-1 through R-15 comprising fade and density results are shown in Tables 5, 6, and 7 below.

TABLE 5

| Element | Shell Polymer and Weight Ratio of Shell to Core | Particle Size microns | Mordant Level (equivalents) | % Magenta Fade From Density 1.0 7 days | % Magenta Fade From Density 1.0 60 ppb O <sub>3</sub> |
|---------|-------------------------------------------------|-----------------------|-----------------------------|----------------------------------------|-------------------------------------------------------|
| C-1     | None                                            | 0.091                 | 1                           | 31.9                                   | 41.1                                                  |
| R-1     | Celvol 203                                      | 0.101                 | 1                           | 7.3                                    | 12.0                                                  |

TABLE 6

| Element | Shell Polymer And Weight Ratio of Shell to Core | Particle Size | Mordant Level (equivalents) | % Magenta Fade From Density 1.0 7 days | % Cyan Fade From Density 1.0 7 days | % Black Fade From Density 1.0 7 days |
|---------|-------------------------------------------------|---------------|-----------------------------|----------------------------------------|-------------------------------------|--------------------------------------|
| C-1     | None                                            | 0.091         | 1                           | 28.3                                   | 23.9                                | 19.2                                 |
| C-2     | None                                            | 0.166         | 1                           | 25.5                                   | 24.2                                | 19.3                                 |
| R-2     | SP-1                                            | 0.282         | 1                           | 19.0                                   | 19.5                                | 16.5                                 |
| R-3     | SP-1                                            | 0.247         | 1                           | 23.0                                   | 20.3                                | 17.3                                 |
| R-4     | SP-1                                            | 0.213         | 1                           | 23.1                                   | 20.9                                | 18.0                                 |

The results in Table 6 show core shell particles with cationic mordanting cores and nonionic polyvinyl alcohol shells reduce the amount of dye fade that results from the exposure of test prints to high concentrations of ozone.

TABLE 7

| Example | Weight Ratio Shell to Core | Shell Polymer | Median Particle Size $\mu\text{m}$ | Mordant Level (equivalents) | % Magenta Fade From Density 1.0 7 days | % Cyan Fade From Density 1.0 7 days | % Black Fade From Density 1.0 7 days |
|---------|----------------------------|---------------|------------------------------------|-----------------------------|----------------------------------------|-------------------------------------|--------------------------------------|
| C-1     | 0:1                        | None          | 0.091                              | 1                           | 61.8                                   | 42.1                                | 36.4                                 |
| C-3     | 0:1                        | None          | 0.091                              | 1.5                         | 56.9                                   | 39.5                                | 34.0                                 |
| R-5     | 2.8:1                      | SP-1          | 0.123                              | 1                           | 43.5                                   | 34.4                                | 28.4                                 |

TABLE 7-continued

| Example | Weight Ratio<br>Shell to Core | Shell<br>Polymer | Median<br>Particle<br>Size $\mu\text{m}$ | Mordant<br>Level<br>(equivalents) | % Magenta<br>Fade From<br>Density 1.0<br>7 days<br>60 ppb $\text{O}_3$ | % Cyan<br>Fade From<br>Density 1.0<br>7 days<br>60 ppb $\text{O}_3$ | % Black<br>Fade From<br>Density 1.0<br>7 days<br>60 ppb $\text{O}_3$ |
|---------|-------------------------------|------------------|------------------------------------------|-----------------------------------|------------------------------------------------------------------------|---------------------------------------------------------------------|----------------------------------------------------------------------|
| R-6     | 2.8:1                         | SP-1             | 0.123                                    | 1.5                               | 43.1                                                                   | 32.3                                                                | 26.0                                                                 |
| R-7     | 1.6:1                         | SP-1             | 0.119                                    | 1                                 | 56.2                                                                   | 40.6                                                                | 31.8                                                                 |
| R-8     | 1.6:1                         | SP-1             | 0.119                                    | 1.5                               | 39.3                                                                   | 29.2                                                                | 24.7                                                                 |
| R-9     | 2.4:1                         | SP-3             |                                          | 1                                 | 37.2                                                                   | 28.5                                                                | 23.0                                                                 |
| R-10    | 2.4:1                         | SP-3             |                                          | 1.5                               | 24.9                                                                   | 17.3                                                                | 10.0                                                                 |
| R-11    | 1.5:1                         | SP-3             |                                          | 1                                 | 43.1                                                                   | 33.1                                                                | 26.7                                                                 |
| R-12    | 1.5:1                         | SP-3             |                                          | 1.5                               | 39.3                                                                   | 29.2                                                                | 24.7                                                                 |
| R-13    | 2.7:1                         | SP-2             | 0.137                                    | 1                                 | 33.9                                                                   | 28.6                                                                | 22.5                                                                 |
| R-14    | 2.7:1                         | SP-2             | 0.137                                    | 1.5                               | 23.2                                                                   | 27.2                                                                | 17.1                                                                 |
| R-15    | 1.5:1                         | SP-2             | 0.128                                    | 1                                 | 52.8                                                                   | 36.4                                                                | 29.1                                                                 |
| R-16    | 1.5:1                         | SP-2             | 0.128                                    | 1.5                               | 45.0                                                                   | 30.7                                                                | 24.8                                                                 |

All of the invention examples in Table 7 show reduced dye fade in comparison with the Example C-1. In general, the amount of protection increases as the shell thickness increases, and it also increases as the amount of core shell mordant is increased. The improvements are observed with all three shell polymer compositions.

The invention has been described in detail with particular reference to certain preferred embodiments thereof, but it will be understood that variations and modifications can be effected within the spirit and scope of the invention.

What is claimed is:

1. An inkjet recording element comprising a support having thereon at least one porous image-receiving layer comprising:

- (a) insoluble cationic core-shell polymeric particles, each comprising a core and a shell, the core comprising a cationic core polymer having at least 10 mole percent of a cationic mordant monomeric unit and the shell comprising hydrophilic shell polymer that is substantially less cationic than the cationic core polymer, wherein the shell is at least 10% by weight of the core; and
- (b) inorganic and/or organic particles other than the insoluble cationic core-shell polymeric particles in a total amount of greater than 50 percent by weight of the porous image-receiving layer, and the weight ratio of the insoluble cationic core-shell polymeric particles to inorganic and/or organic particles in the image-receiving layer is 1:2 to 1:20.

2. The inkjet recording element of claim 1 wherein the hydrophilic shell polymer is at least 50 percent less cationic than the cationic core polymer, in terms of number of cationic groups per weight average molecular weight of the polymer.

3. The inkjet recording element of claim 1 wherein cationic groups are essentially absent from the hydrophilic shell polymer.

4. The inkjet recording element of claim 1 wherein the cationic core polymer comprises styrenic polymer, acrylic polymer, or polyester polymer.

5. The inkjet recording element of claim 1 wherein the cationic core polymer is between 0.5 and 15 mole percent of a monomer capable of crosslinking.

6. The inkjet recording element of claim 1 further comprising one or more ink-retaining layers or base layers under one or more image-receiving layers and an optional overcoat.

7. The inkjet recording element of claim 1 wherein the hydrophilic shell polymer is chemically bonded to the cationic core polymer.

8. The inkjet recording element of claim 7 wherein the hydrophilic shell polymer is chemically bonded to the cationic core polymer through an amine linking group.

9. The inkjet recording element of claim 8 wherein the amine linking group is attached to the cationic core polymer at a monomeric location in the cationic core polymer, elsewhere occupied by a quaternary amine group.

10. The inkjet recording element of claim 1 wherein the inorganic particles are selected from the group consisting of fumed and/or colloidal particles.

11. The inkjet recording element of claim 10 wherein the inorganic particles are selected from the group consisting of fumed silica, fumed alumina, colloidal silica and/or hydrated alumina, boehmite and other hydrated alumina, and combinations thereof.

12. The inkjet recording element of claim 1 wherein the cationic core polymer comprises quaternary ammonium salt moieties.

13. The recording element of claim 1 wherein the cationic core polymer, in the insoluble cationic core-shell polymeric particles, comprises monomeric units selected from the group consisting of (vinylbenzyl)trialkyl quaternary ammonium salt, (vinylbenzyl)dialkylbenzyl quaternary ammonium salt moiety, and combinations thereof, wherein the alkyl groups have 1 to 6 carbon atoms.

14. The recording element of claim 1 wherein the insoluble cationic core-shell polymeric particles have a mean particle size of from about 10 to about 500 nm.

15. The recording element of claim 1 wherein the at least one image-receiving layer further contains a hydrophilic binder in an amount of 3 to 20 weight percent.

16. The inkjet recording element of claim 1 wherein the hydrophilic shell polymer comprises hydroxy, ether ketone, nitrile, and/or amino acid groups.

17. The inkjet recording element of claim 16 wherein the hydrophilic shell polymer is selected from the group comprising poly(vinyl alcohol) or a copolymer, or derivative thereof, and gelatin.

18. The inkjet recording element of claim 1 wherein the hydrophilic shell polymer is characterized by a  $p(\text{O}_2)$  of less than  $25 \text{ cm}^3 \cdot \mu\text{m}/\text{m}^2 \cdot \text{day} \cdot \text{Kpa}$ .

19. An inkjet printing method using an image-recording element, which provides an image having excellent image quality and superior dry time and comprising the steps of:

- a) providing an ink printer that is responsive to digital data signals;
- b) loading the printer with an image-recording element comprising a support having thereon at least one porous

**31**

image-receiving layer, comprising insoluble cationic core-shell polymeric particles, in an amount effective for mordanting a dye-based ink in printed images, each core-shell polymeric particle comprising a core and a shell, a core comprising insoluble cationic core polymer having at least 10 mole percent of a cationic mordant monomeric unit and a shell comprising hydrophilic shell polymer that is substantially less cationic than the insoluble cationic core polymer, wherein the shell is at least 10% by weight of the core, and the weight ratio of

5

**32**

the cationic core-shell polymeric particles to other particles in the image-receiving layer is 1:2 to 1:20;  
c) loading the printer with an ink composition; and  
d) printing on the image-recording element using the ink composition in response to the digital data signals.

**20.** The method of claim **19** wherein the cationic mordant monomeric unit comprises a quaternary ammonium, pyridinium, or imidazolium moiety.

\* \* \* \* \*

UNITED STATES PATENT AND TRADEMARK OFFICE  
**CERTIFICATE OF CORRECTION**

PATENT NO. : 7,833,591 B2  
APPLICATION NO. : 11/617777  
DATED : November 16, 2010  
INVENTOR(S) : Ghyzel et al.

Page 1 of 1

It is certified that error appears in the above-identified patent and that said Letters Patent is hereby corrected as shown below:

In Column 30, line 41, claim 13 delete “(vinylbenzyl)trialkyl” and insert -- (vinylbenzyl)trialkyl --.

Signed and Sealed this  
Twelfth Day of April, 2011



David J. Kappos  
Director of the United States Patent and Trademark Office